

Dec. 12, 1950

C. E. DILL

2,533,228

METHOD OF CALENDERING SHEET MATERIAL

Filed Oct. 12, 1946

FIG.1



INVENTOR.

Charles E. Dill  
by  
Walter J. Caulfield  
attorney

## UNITED STATES PATENT OFFICE

2,533,228

## METHOD OF CALENDERING SHEET MATERIAL

Charles E. Dill, Dover, N. J., assignor to Armstrong Cork Company, Lancaster, Pa., a corporation of Pennsylvania

Application October 12, 1946, Serial No. 702,966

7 Claims. (Cl. 117—111)

1

This invention relates to a method of applying a film of lubricant to calender rolls to prevent sheet material passing therebetween from adhering to the rolls, and to apply a film of wax to the surface of the sheet material.

An object of this invention is to provide a means for preventing asphalt tile sheets or other thermoplastic sheets from adhering to the hot calender roll during the sheet finishing operation. A further object is to produce a flooring tile having a surface free from "chill marks" or small breaks. A still further object is to apply a coating of wax to the surface of the tile at the time it passes through the finishing calender, thereby eliminating the subsequent waxing operation in the manufacture of flooring tile of this kind.

The use of lubricants to prevent calendered sheets from adhering to the calender rolls is old in the art of manufacturing sheet material, but the lubricating oil usually used for this purpose is not satisfactory for the manufacturing process here under consideration due to the fact that the binder for the thermoplastic sheet material is compatible with the lubricating oil. This causes a certain amount of binder to be dissolved in the oil resulting in defective material due to the fact that only a partial amount of the required binder remains in the finished product.

Attempts have been made to produce asphalt tile by means of cold calender rolls (below 130° F.). This process prevents the sheets from adhering to the rolls but the cold roll produces "chill marks" on the surface of the tile sheets. These "chill marks" are actually small cracks or breaks in the surface of the tile and are highly undesirable in the wear surface of hard surface floor covering. Furthermore, it has been customary in the past to apply a film of wax to the finished material before it is packaged for shipment to the dealer. This requires another step in the process of manufacturing asphalt tile.

By my invention it is possible to make asphalt tile from the usual thermoplastic mass and pass it through a calender having a heated facing roll. This is accomplished by spraying a film of wax emulsion on the heated roll. The binder used in asphalt tile composition is not water-soluble and, therefore, any small amount of water remaining in the wax emulsion has no effect upon the binder. Furthermore, the wax emulsion used to prevent the sheets from adhering to the calender roll remains on the surface of the sheet material and serves as a wax coating to protect the wear surface of the flooring material.

In the manufacture of asphalt tile, the ingre-

2

dients are thoroughly mixed in an internal mixer, at the completion of which the loose thermoplastic mix is dumped into a sheeting calender, one roll of which operates at about 325° F., and the other of which operates at about 180° F. This sheeting calender performs the step of initial heat consolidation of the loose mass into sheet form. A suitable scraper or doctor blade is provided to free the sheets from the hot roll on this initial heat consolidating calender. From this initial sheeting calender, the sheets travel by means of a suitable conveyor to a second calender known as a finishing or facing calender, the top roll of which is maintained at between 180° and 250° F. and the bottom roll of which is maintained at about 130° F. This finishing or facing calender effects final heat consolidation of the thermoplastic mass. The temperature at which the hot roll on this finishing calender operates is sufficiently high to cause the surface of the sheets to adhere to the roll. The bottom roll or cold roll is operated at a temperature sufficiently low to prevent the sheet from adhering thereto.

To overcome the problem of the sheets adhering to the hot roll, I have arranged a series of sprayer nozzles suitable for spraying a film of aqueous wax emulsion to the surface of the roll. In addition to this sprayer device, a wiper is provided to evenly distribute the aqueous wax emulsion in a film of uniform thickness throughout the width of the roll. This lubricated roll serves as the finishing roll or facing roll in the final calendering operation and the lubricated surface thereof prevents the face of the sheets from adhering to the calender roll. Also, the lubricated roll transfers a film of lubricant to the surface of the sheet being calendered. The thermoplastic sheet material as it passes through the finishing calender is at a temperature of approximately 250° F. Inasmuch as this temperature is substantially above the boiling point of the water in the wax emulsion, the water is boiled off, leaving a film of wax on the surface of the sheet material.

After this final calendering operation, the sheets pass through a cooling zone and then a dieing operation which forms the asphalt tile to the desired size and shape.

The accompanying drawing shows a diagrammatic view of an asphalt tile calender suitable for carrying out the process of my invention. In this drawing, 2 is a conventional facing roll or hot roll which is maintained at a temperature of between 180° F. to 250° F. A series of suitable spray nozzles, indicated at 4, is provided for applying a film of wax emulsion to the surface

of the hot roll. I have found that it is difficult to obtain an even film of wax by means of the spray nozzles. To overcome this difficulty, I provide a wiper, shown at 5, to spread the wax evenly across the entire width of the roll. For best results, the wiper should be placed about 75° back of the series of spray nozzles. It is essential that the wax be disposed uniformly on the roll, not only to prevent particles from adhering to all areas of the roll but to transfer a uniform film of wax to the face of the calendered tile. The cold roll, indicated at 3 in the drawing, is usually maintained at a temperature of approximately 130° F. At this low temperature, there is no tendency for the sheet material to adhere to the surface of the roll 3.

At 6 there is shown a belt conveyor suitable for delivering the unfinished sheet material to the calender rolls and 7 indicates a belt conveyor suitable for carrying the finished waxed sheets away from the finishing calender to the subsequent dieing operation.

In carrying out the process of my invention, the best results have been obtained by use of the sprayer-wiper combination explained above, although the invention can be carried out in various other ways such as the use of a wick for applying wax emulsion to the rolls. Also the wax emulsion may be dropped on the roll by gravity instead of by the sprayer system.

Several of the commercially obtainable wax emulsions have been found to be satisfactory in carrying out the process of my invention, but I have found the best results to be obtained with an emulsion of the following formulation:

|                                                             | Pounds |
|-------------------------------------------------------------|--------|
| Carnauba wax                                                | 100    |
| Triethanolamine                                             | 14     |
| Borax                                                       | 6      |
| White oleine                                                | 14     |
| Sufficient water to form an emulsion containing 15% solids. |        |

While the above formulation is preferred for carrying out my invention, it will be understood, of course, that other waxes in emulsion form may be employed satisfactorily.

I have found the best results to be obtained with a wax emulsion having a solids content of 15%, however, satisfactory results are obtained with solids content ranging from 12½% to 25%. If more than 25% solids are present in the emulsion, there is a tendency for the wax to build up on the roll rather than be transferred from the roll to the surface of the sheet material. Also, if an emulsion containing a greater percentage of solids is used, the wiper becomes clogged and does not perform its proper function in distributing the wax emulsion uniformly across the surface of the roll. If the emulsion contains less than 12½% solids, it does not prevent the surface of the sheet material from adhering to the calender roll, and, furthermore, the wax film remaining on the wear surface of the tile is not sufficiently heavy to properly protect the tile.

In the manufacture of asphalt tile in accordance with the process outlined above, the difficulty of the face of the tile sticking to the hot roll has been eliminated and the finished tile has a substantially smooth wear surface free from "chill marks" and other defects which usually arise when a cold roll is used as a facing roll for this material. In addition to this advantage, the sheet material has a film of wax applied to the wear surface thereof at the time it passes through the

finishing calender. This eliminates the necessity for having a separate operation to perform this step in the process of manufacturing asphalt tile or similar flooring materials.

While I have described and illustrated certain preferred embodiments of my invention, it will be understood that the invention may be otherwise embodied and practiced within the scope of the following claims.

I claim:

1. In a method of forming a sheet from a thermoplastic mass, the steps comprising delivering to the nip between a pair of calendering rolls a mass of thermoplastic material heated to a temperature above 212° F., at which said heated mass is plastic and may be sheeted by calendering, the face-forming roll of said calender being maintained at a temperature at which said heated mass would normally adhere under consolidating pressure in sheet formation, interposing a film of an aqueous wax emulsion between the surface of the face-forming roll and said heated mass under treatment, said heated mass being non-adherent to said face-forming roll with said interposed film under consolidating pressure in sheet formation, consolidating said mass into a sheet between said rolls with said film of aqueous wax emulsion interposed between said face-forming roll and said heated mass, removing water from said wax emulsion film by the application of heat thereto from said heated mass under consolidation, and removing the formed and wax coated sheet from said calender rolls substantially free of cracks or breaks in the face thereof.
2. A method in accordance with claim 1 in which the aqueous wax emulsion is sprayed on the face-forming roll to form a film thereon and in which a portion at least of the film is transferred from the face-forming roll to the face of the consolidated sheet during consolidation and sheet formation.
3. A method in accordance with claim 1 in which the aqueous wax emulsion contains from 12½% to 25% of solids.

4. A method in accordance with claim 1 in which the face-forming roll is maintained at a temperature between 180° F. and 250° F.

5. A method in accordance with claim 4 in which the mass of thermoplastic material delivered to the nip between the calender rolls is heated to a temperature of about 250° F.

6. A method in accordance with claim 1 in which the aqueous wax emulsion comprises by weight 100 parts carnauba wax, 14 parts triethanolamine, 6 parts borax, 14 parts white oleine, and sufficient water to form an emulsion containing from 12½% to 25% solids.

7. A method in accordance with claim 1 in which the aqueous wax emulsion contains about 15% solids.

CHARLES E. DILL.

#### REFERENCES CITED

The following references are of record in the file of this patent:

#### UNITED STATES PATENTS

| Number    | Name           | Date          |
|-----------|----------------|---------------|
| 1,312,682 | Clapp          | Aug. 12, 1919 |
| 1,590,638 | Marquette      | June 29, 1926 |
| 1,698,267 | Kirschbraun    | Jan. 8, 1929  |
| 2,025,375 | Cameron et al. | Dec. 24, 1935 |
| 2,177,240 | Brumbaugh      | Oct. 24, 1939 |
| 2,349,326 | Wilson         | May 23, 1944  |